# EUROPEAN PATENT SPECIFICATION

(11) **EP 3 027 342 B1**
(45) Date of publication and mention of the grant of the patent: **03.03.2021**
(21) Application number: 14749941.2
(22) Date of filing: 01.08.2014
(51) Int. Cl.: B22D 23/06, B22D 27/04

(54) **FORMING A METAL COMPONENT**
HERSTELLUNG EINES METALLISCHEN BAUTEILS
FORMAGE D'UN ÉLÉMENT MÉTALLIQUE

(30) Priority: 02.08.2013 GB 201313849; 15.11.2013 GB 201320168; 15.11.2013 GB 201320171
(43) Date of publication of application: 08.06.2016
(73) Proprietor: Castings Technology International Ltd., Sheffield, South Yorkshire S10 2TN (GB)
(72) Inventor: ASHTON, Michael Cornelius, South Yorkshire S17 4QB (GB); COLLINS, James Michael, Doncaster DN2 5SD (GB)
(74) Representative: Harkness, Katherine Joy
(86) International application number: PCT/GB2014/000303
(87) International publication number: WO 2015/015144

(56) References cited:
- EP-A2- 0 708 187

## Description

### BACKGROUND OF THE INVENTION

### 1. Field of the Invention

The present invention relates to a method of forming a metal component from a powdered feed material.

The present invention also relates to an apparatus for forming a metal component from a powdered feed material.

### 2. Description of the Related Art

Powder metallurgy is a known method for forming a metal component, from a powdered feed material. In a known hot isostatic pressing (HIP) process, powder is shaped in a steel mould to which both pressure and temperature are applied. Typically, argon gas is used to provide the isostatic pressure which may range from 50 megapascal to 300 megapascal. During this process, the temperature of the material is raised so as to sinter the powder and cause the particles to fuse together. However, known powder metallurgy is limited in terms of the size of products that can be produced and also in terms of the complexity of their shape. Furthermore, it is a costly and time consuming process. It is difficult to scale and often impossible to produce products having the required size and complexity when competing against products produced by a more conventional casting process.

European Patent No. 0 708 187 discloses a method and apparatus for directional solidification of a melt. Refractory particulates are provided about at least one region of a casting mould and are heated using an induction heating system and a susceptor element. Heat is then conducted from the particles to the mould.

### BRIEF SUMMARY OF THE INVENTION

According to a first aspect of the present invention, there is provided a method of the aforesaid type for forming a metal component from a powdered feed material, comprising the steps of: creating a negative mould of a component from a ceramics material having a melting point that is higher than the melting point of said powdered feed material; deploying said feed material of metal powder into said mould; locating said mould in a vacuum chamber having an induction or microwave heating system, said heating system comprising a source of electromagnetic energy and a granular susceptance material; and heating said mould using said induction heating system to a temperature higher than the melting point of the metal powder so as to melt the metal powder within the mould; wherein said granular susceptance material absorbs the energy of the induction field generated by said source of electromagnetic energy and radiates infra-red energy towards the ceramic mould. In an embodiment, during the deployment of the feed material into the mould, a degree of vibration may be introduced to facilitate the dispersal of the feed material within the mould.

According to a second aspect of the present invention, there is provided an apparatus for forming a metal component from a powdered feed material, comprising: a negative mould of a component comprised of a ceramics material having a melting point higher than the melting point of said powdered feed material contained therein; and a vacuum chamber for receiving said mould, the vacuum chamber being having a microwave or induction heating system comprising a source of electromagnetic energy and a granular susceptance material; wherein said granular susceptance material configured to absorb the energy of the induction field generated by said source of electromagnetic energy and radiate infra-red energy towards the ceramic mould.

### BRIEF DESCRIPTION OF THE DRAWINGS

Figure 1 shows a method of forming a metal component;
Figure 2 shows procedures for the creation of a positive model;
Figure 3 shows the addition of layers to produce a mould;
Figure 4 shows the deployment of feed material;
Figure 5 shows apparatus for forming a metal component;
Figure 6 shows a cross section of a feeder section;
Figure 7 shows the mould of Figure 5 after being loaded with metal powder;
Figure 8 shows the mould of Figure 7 with liquid metal;
Figure 9 shows a partial cross section view of the mould;
Figure 10 shows the view of Figure 9 after further cooling;
Figure 11 shows a mould of an alternative configuration;
Figure 12 illustrates a heating system;
Figure 13 shows an alternative embodiment of the mould; and
Figure 14 shows a mould immersed in a granular susceptance material.

### DETAILED DESCRIPTION OF EXAMPLE EMBODIMENTS

### Figure 1

A method of forming a metal component from a powdered feed material is illustrated in Figure 1. A feed material is initially in a powdered state (detailed in Figure 4) and a solid component is formed by the application of heat (detailed in Figure 12). At step **101** a sacrificial positive model **102** of a component is created. At step **103,** a negative mould **104** is built around the positive model from a material having a melting point higher than the melting point of the material from which the component is to be formed (as detailed in Figure 3).

At step **105** the sacrificial positive model is removed so as to leave a void **106** within the negative mould.

At step **107** feed material of metal powder **108** is deployed into the mould. At step **109 heat 110** is applied to the mould to a temperature higher than the melting point of the metal powder so as to cause the metal powder to melt within the mould, thereby establishing molten metal **111** within the mould **104.**

The metal powder **108** used herein to form a metal component is, in a first embodiment, a powder consisting of particles of pure metal. However, in an alternative embodiment metal powder **108** is a powder comprising particles of an alloy. It should be appreciated therefore, that metal components formed from the said metal powder may be comprised either of a pure metal or an alloy compound.

Whereas metal powders need to be graded to specific size ranges for known powder metallurgy techniques, such as HIPping, powder metallurgy, metal injection moulding, etc, the method described herein is relatively insensitive to the size range of the powder particles. The only requirement is that the metal powder flows readily into the ceramic moulds. Where the mould defines sections having diameters as little as 0.5 millimetres, spherical powders produced by gas atomisation, for example, would be more appropriate. With larger mould sections, even angular powders produced by crushing and milling would enable the mould to be filled, especially when the flow of powder is aided by vibration, as will be described with reference to Figure 4.

### Figure 2

Procedures for the creation of the positive sacrificial model are illustrated in Figure 2. Operations are performed upon a source material **201** in order to produce the positive model **102.** In a first embodiment, it is possible to perform a machining operation **202** upon an appropriate material in order to define the shape of the positive model. However, it should be appreciated that the material used must be of a type such that it is possible to remove the sacrificial material in order to define the negative mould.

As an alternative, it is possible to perform a wax injection process **203.** Having created a mould around the wax positive, it is possible to remove the wax by the application of heat. Such an approach is known in conventional casting systems where the heating of the mould is also desirable prior to the application of molten metal. However, in an embodiment, the mould would be allowed to cool and the particulates would be added at room temperature.

As an alternative, it is also possible to produce the positive mould by a process of additive manufacturing **204,** with an appropriate rapid prototyping material for example. The material may be removed by the application of heat and/or the application of an appropriate solvent.

### Figure 3

In the embodiment, the negative mould, having a melting point higher than the melting point of the metal from which the component is to be formed, is a ceramic shell that is relatively porous to air. In an embodiment, the ceramic mould is produced by adding a plurality of layers, as shown in Figure 3.

In the embodiment shown in Figure 3, layers are added as an alternating wet slurry layer followed by a substantially dry stucco layer.

Slurry **301** is applied to the model **102.** Dry stucco **302** is then applied that attaches itself to the wet slurry in order to build a layer.

This process is repeated, as shown generally at **303,** resulting in the build up of a layer **304.** Thus, further repetitions are made until the negative mould **104** has been built to the required thickness. Ceramic mould 104 should ideally have relatively thin wall sections so as to allow the conduction of radiant heat from a radiant heating system therein, to enable the metal powder to be melted. However, the wall sections must be sufficiently thick to prevent cracks or fracturing during processing, and therefore a compromise must be reached in creating a mould that has a high thermal conductivity, but is sufficiently strong.

In an embodiment, a primary refractory slurry is applied that is inert to the metal being used. A dry sand of similar or different material is then applied and further slurries are applied, followed by sand, stucco and so on.

A number of suitable ceramic materials for forming the ceramic shell are known, such as silica and alumina. It has been found during testing that a silica shell does not have a sufficiently high thermal conductivity to allow the powder metal charge to be melted in a suitable time-frame using a radiant heating system. Therefore, in a preferred embodiment, a negative mould comprised of an alumina material having a high thermal conductivity is used. Other types of shell material having a high thermal conductivity may be used, however they must not be susceptible to dissolution in the molten metal as can be experienced by graphite based moulds when used certain metals.

### Figure 4

Step **107** for the deployment of feed material is detailed in Figure 4. The positive sacrificial model **102** has been removed as illustrated by step **105.** The negative mould **104** is placed upon a vibrating table **401,** itself supported by a stable base **402.** In this way, as the feed material **108** is deployed into the mould **104,** or after deployment, a degree of vibration is introduced, as illustrated by arrows **403** and **404,** to facilitate the dispersal of the feed material within the mould. High frequency vibration, e.g. 40-60 hertz, with low amplitude displacement of, say, 0.10-0.15 millimetres enables moulds for large and complex metal components to be filled easily.

Thus, the feed material is deployed within the mould and then heated, as illustrated by step **109.** In an embodiment, the heat is applied without pressure and the mould is heated to a temperature that causes the feed material to melt. In this way, it is possible to obtain close to 100 percent density using a process that has less overall complexity compared to known systems. The heat is required not only to raise the temperature of the metal, but also to melt the metal completely. Consequently, it is typically heated to around 50 degrees Celsius above the melting point of the metal, in the case of a pure metal, or above the liquidus temperature in the case of an alloy.

In some known systems, contamination is often introduced from containers and this is a particular problem when using titanium. Processes using solid state diffusion result in the container experiencing a similar environment to the material contained inside. Thus, even after machining away, it is possible that a significant layer of a material mixture will remain. Consequently, additional processing is required in order to achieve the required result.

It has been recognised that the use of metal powder as a feed material may produce products having desirable properties. There is a tendency for the microstructure to be very uniform, which may improve strength and fatigue properties. Properties of this type may be provided by forging operations but, as is known, forging results in the production of significant levels of waste and therefore increases overall cost. Similarly, a casting process yield is typically 50 percent; again increasing cost, which becomes an important factor when expensive alloys are being used.

### Figure 5

An apparatus for forming a metal component from a powdered feed material is illustrated in Figures 5 through 12. As previously described, a sacrificial positive model is created and a negative mould is built around the positive model from a material having a melting point higher than the melting point of the metal from which the material is formed. Thus, this results in the creation of a negative mould, preferably a ceramic mould 501.

The sacrificial positive model is removed from the negative mould 501. The apparatus further comprises a deploying device for deploying the feed material of metal powder into the mould **501,** and a heating system for heating the metal powder to a temperature higher than the melting point of the metal powder so as to cause the metal powder to melt within the mould.

An example of a mould **501** is illustrated in Figure 5 in cross-section. The mould **501** includes a component section **502** corresponding to the component to be produced and a feeder section **503.** The feeder section **503** defines a generally cylindrical passageway **504,** that may include an inwardly extending element as detailed in Figure 6. The feeder section adjoins said component section at a first end and extends vertically upwards towards a distal end that is open to allow insertion of feed materials up to a head level.

The feeder section is provided because when metals cool from their molten liquid state, their volume decreases as the temperature drops to the point where they are solid. Thus, the feeder is used to provide additional liquefied metal to the mould to compensate for the shrinkage cavities that would otherwise form at one or more thermal centres in the interior of the casting as it cools. The volume of the feeder is therefore determined by the requirement for sufficient liquid metal to be provided in order to compensate for the volume reduction of the metal as it cools. Two factors influence the efficiency of feeding; firstly, the metallostatic pressure in the feeder, and secondly the pressure being applied to the liquid metal surface of the feeder by the surrounding atmosphere. The metallostatic pressure head in the feeder assists in forcing the molten metal into the mould section, as metal contained in the mould section cools and decreases in volume.

The head of molten metal should remain molten at least until the metal in the component section has solidified completely. To inhibit the conduction of thermal energy from within the feeder section to outside the feeder section during cooling and to thereby maintain the metal in the feeder in its molten state, the walls of the feeder section should have a relatively lower thermal conductivity than the walls of the component section. The feeder section may therefore be comprised of a different ceramic material to said component section and may comprise insulating or exothermic ceramic powders. Alternatively, the feeders may be wrapped in insulating material to ensure they solidify later than the metal component and to ensure that the surface of the molten metal in the feeder head remains molten so that any atmospheric pressure effects will assist in feeding.

To maximise the metallostatic pressure, the feeder head should be raised as high as is practically and economically feasible in order to maximise the metallostatic pressure,

To further improve the degassing of molten metal in the component section and to increase the pressure applied to the molten metal, one or more atmospheric cores may be provided extending downwardly through the feeder section towards the component section. These atmospheric cores may be pencil shaped ceramic tubes which are porous to gasses and whose permeability allows atmospheric pressure to be applied to the liquid metal in the thermal centre of the feeder section, and to allow gas trapped within the liquefied metal to escape. A particular atmospheric core in the form of an inwardly extending element is described further with reference to Figure 6.

In an embodiment, the ceramic mould is initially at room temperature, therefore it is at a known and relatively constant temperature; compared to situations where the mould may have been heated and the actual temperature of the mould, when material may be added, may fall within a relatively wide range of possible temperatures. However, in an embodiment where the temperature is known in terms of an initial temperature and a melt temperature, it is possible to accurately calculate the volume of powder required in the feeders. Thus, an optimum amount of material may be held in the feeders so as to compensate for the 30-35 percent contraction in volume during the overall process.

A cross-sectional view of the mould through horizontal plane **503** is illustrated in Figure 6.

### Figure 6

The feeder section **503** defines a generally cylindrical passageway **504.** The passageway **504** includes an atmospheric core, here provided by inwardly extending element **505** that is porous to gasses and extends inwardly from the generally cylindrical inside surface **506** of the passageway **504** defined by the feeder towards the middle of the cylindrical passageway. In an embodiment, the inwardly extending element **505** is substantially wedge-shaped, having faces arranged at an acute angle to each other, to form a sharp edge **507** close to the middle of passageway **504** and is formed of the same porous material from which the feeder is formed.

In an embodiment the mould is located within the chamber of a vacuum furnace in order to melt the metal powder within the mould. During this process, the inwardly extending element provides a means for allowing the atmosphere in the chamber to access molten metal in the feeder during cooling of the metal component, to allow gas trapped within the molten material to be released. The inwardly extending element therefore functions as an atmospheric core whose permeability allows pressure to be applied to the liquid metal in a thermal centre of the feeder head and to allow gas to escape from the molten metal in the component and feeder sections of the mould.

### Figure 7

Mould **501** is shown in Figure 7, after being loaded with metal powder **108** during process **107.** The metal powder has been poured into an open end **702** of the feeder **503** up to a head level, and vibrated (as described with reference to Figure 4) to compact the metal powder **108.** In an embodiment, the feeder is filled with metal powder to the top of said feeder. The mould is then vibrated, resulting in the upper surface **703** of the metal powder in the feeder becoming lower, when compared to the level of the powder before vibration.

In an embodiment, the metal powder is formed from substantially spherical particles. Consequently, even after compaction by vibration, approximately 25-30 percent of the volume taken up by the powder 108 comprises voids between the particles. In an alternative embodiment, other shapes of particles may be deployed, either alone or in combination with spherical partials. The inclusion of particles of this type may decrease the volume taken up by voids within the powder.

### Figure 8

Mould **501** is shown in Figure 8, after the metal powder **108** has melted to form a liquid metal **801.** An upper surface **802** of the liquid metal has gone down the feeder when compared to the surface **703** of the powder. However, in this embodiment, the height of the molten metal **801** in the feeder is greater than twice the height of the section of the mould corresponding to the metal object being produced. The height of the component section of the mould corresponding to the component to be produced is indicated by arrow **803** and the height of the molten metal 801 in the feeder section **503** is indicated by arrow **804.** Thus, in this embodiment, the height indicated by arrow **804** is more than twice the height of that indicated by arrow **803.**

A pressure is created within the molten metal due to the weight of molten metal in the feeder. By introducing a relatively high feeder of molten metal, sufficient pressure may be produced in the molten metal within the mould to ensure that the molten metal is forced into fine details of the mould surface.

### Figure 9

A partial cross-sectional view of the mould **501** is illustrated in Figure 9. As the mould cools, heat is conducted from the molten metal through the walls of the mould. Consequently, the outside of the molten metal tends to solidify first, with the solidification process continuing in an inward direction.

In the example of Figure 9, region **901,** adjacent to the walls of the mould, is in the process of crystallizing, whereas portions of the metal away from the walls are still liquid. During solidification, the metal contracts typically by about 7 percent by volume and consequently voids **902** form within the molten metal.

### Figure 10

When voids are surrounded by molten metal, metal will tend to fall into the void under gravity, resulting in voids appearing to rise up the mould.

In an embodiment, the feeder is arranged such that the voids rise into the feeder and metal within the feeder falls into the mould to ensure that the mould is completely filed.

In the example shown in Figure 10, voids **902** have coalesced to form a single void **1001** that has risen up to the feeder.

Generally, voids, such as void **1001,** will define a volume of space containing a vacuum. However, these voids may contain some gas that has become trapped by the molten metal within the mould. In an embodiment, the inwardly extending element **505** provides a means for allowing gas trapped within the molten metal in the feeder to escape. The inwardly extending element is able to do this because it is a relatively good insulator of heat (compared to the metal itself) and it extends into the molten core of the metal within the feeder. Furthermore, the element is porous to gases.

### Figure 11

The mould described with reference to Figures 5 through 10 has a single feeder that provides a means of receiving powder into the mould, while also providing a metallostatic head for producing an elevated metallostatic pressure in the mould. However, in an alternative embodiment, one or more additional feeders may be provided; separate from the feeder providing the metallostatic head pressure.

An example is shown in Figure 11 in which a mould **1101** has a lower section **1102** corresponding to the metal object to be produced. In addition, the mould has a first feeder **1103,** a second feeder **1104** and a third feeder **1105.**

The second feeder **1104** is substantially similar to the feeder **503** shown in Figure 5, having a height that is more than twice the height of section **1102** and providing an opening **1106** at its upper end for receiving powdered metal **1107.**

The first feeder **1103** and the third feeder **1105** are similar to feeder **1104** but differ in that their heights are substantially less than the height of the second feeder **1104.** Furthermore, their upper ends have been capped such that said ends are completely sealed.

The first feeder **1103** and the third feeder **1105** contain powdered metal for feeding section **1102.** They also define a passageway, for receiving voids formed in the molten metal during the cooling process. However, the metallostatic pressure is provided by the second feeder **1104.** Initially open feeders may be formed on moulds and subsequently sealed by a cap that is cemented in place. Alternatively, the feeders may be formed during the manufacture of the mould with a sealed upper end.

### Figure 12

An embodiment of an apparatus for forming a metal component from a powdered feed material is shown in Figure 12. In the embodiment, the induction heating system includes a source of electromagnetic energy, such as coil **1207** for generating radio frequency energy from an electrical supply, along with a control circuit for controlling the electrical supply in order to control temperature. The apparatus further comprises a granular susceptor material, which is in this embodiment contained with the walls of moulds **501.**

A granular susceptor is a preferred form of susceptor material as it enables the susceptor to be contoured to the shape of the mould to which heat is to be applied. In an embodiment a refractory tube is formed of a ceramic material in a shape corresponding to the shape of the mould it heats. The tube is then filled with a granular susceptance material which acts to radiate heat to the adjacent mould. This provides a very versatile susceptor element, which is not otherwise possible when using a solid susceptor ingot which is hard to machine to an appropriate shape. In a specific embodiment, discussed with reference to Figure 14, the granular susceptor material forms a loose bed into which the mould is wholly immersed, thereby ensuring intimate contact between susceptor and mould and an efficient transfer of thermal energy.

An embodiment of the invention further includes pressure reduction apparatus configured to reduce the pressure of a chamber to a pressure below atmospheric pressure. An example of this apparatus is shown in Figure 12. Pressure reduction is desirable in order to reduce contamination from the surrounding atmosphere. However, although extremely low pressures are possible, vapour pressure is required within the chamber in order to prevent evaporation of the molten material.

The apparatus, indicated generally at **1201,** has a vacuum furnace **1202.** The vacuum furnace has a vacuum-tight vessel **1203,** with a refractory lining **1204,** defining a vacuum chamber **1205.**

Vessel **1203** is provided with a door **1206,** for the purpose of providing access to the chamber **1205,** thereby allowing the chamber to be loaded and unloaded with moulds, such as mould **501.**

In an embodiment, the vacuum furnace **1202** has a radio frequency coil 1207 connected to a suitable electrical power supply **1208.** Typically, radio frequency coils are formed of molybdenum, but the full specification of the vacuum furnace will depend upon the specific types of metals and alloys that are being used in the process. Furthermore, the specification will also depend upon the requirements of the metal objects that are being formed.

In an embodiment, the vacuum furnace, its radiation source and power supply are selected such that the temperature of the chamber may be raised to a temperature in excess of 2000 degrees Celsius. Furnaces with these capabilities are commercially available, generally for the purpose of providing heat treatment operations.

Chamber **1205** is connected to a vacuum system **1209** for evacuating air from the chamber, such that pressures in the chamber may be reduced to levels substantially below atmospheric pressure.

The chamber **1205** has an inlet port **1211** connected to a noble gas supply. In an embodiment, a tank **1212** of compressed helium may be provided in combination with a tank **1213** of compressed argon.

The apparatus **1201** also includes a fan **1214** having an inlet connected to outlet port **1210** of chamber **1205** and an outlet connected to the inlet port **1211.** In an embodiment, helium gas is supplied to the chamber **1205** up to a predetermined pressure and the gas is circulated by the fan **1214** to provide a cooling draft over the moulds contained in the chamber.

Temperature sensors **1215** are located within the chamber and in preferred embodiments placed in contact with the moulds so as to provide signals indicative of an actual temperature of the powdered or molten metal in the moulds located within the chamber. The apparatus also includes a vacuum pressure gauge **1216** configured to provide an indication of vacuum pressure within the chamber.

In an embodiment, the pressure gauge **1216** and the temperature sensor **1215** are arranged to provide signals to a controller **1217** indicative of the pressure and temperature of the chamber. The controller is arranged to operate the power supply **1208** for the resistance heating element **1207** and the vacuum system **1209,** in response to the signals received from gauge 1216 and sensor **1215.** In an embodiment, controller **1217** is a programmed computer system or a microcontroller.

### Figure 13

An alternative embodiment of the present invention is illustrated at **1301** in Figure 13. To form a metal component, a mould **1302** is filled with metal particles **1303.** A source **1304** of electro-magnetic radiation is provided and a susceptance material is configured to be heated in response to receiving electro-magnetic radiation and to thermally heat the metal particles **1303.** it has been determined that when heating a metal powder in a ceramic mould using induction heating, the induction field couples too weakly with the powder metal itself to melt it. The ceramic mould of the present invention, unlike a conventional metal mould is relatively transparent to the induction field and is therefore not itself heated. Therefore, when heating using an induction field, a radiant susceptor is preferred. The susceptor is chosen to be of a material so that it absorbs the energy of the induction field and radiates infra-red energy towards the ceramic mould. This causes the ceramic mould to be heated, which in turn heats the metal powder contained within.

In an embodiment, the electro-magnetic radiation is microwave radiation and said apparatus further comprises a source of microwave radiation, in the form of a microwave generator. Microwave radiation is a preferred type of energy as it is efficiently generated and easily guided. When using microwave energy a preferred susceptor material is silicon carbide. Silicon carbide is less prone to thermal degradation than many other susceptor materials and it can typically be heated to temperatures in excess of 3000 degrees Celsius. In the embodiment shown at **1301,** the granular susceptance material is included in the mould **1302** itself however, it is possible for a granular susceptor mass to be provided separately, in a configuration substantially similar to that shown in Figure 14.

### Figure 14

An alternative embodiment for forming a metal component is shown at **1401.** A mould **1402** receives metal particles **1403.** A source **1404** emits electro-magnetic radiation directed towards a container **1405.** The container **1405** is substantially transparent to the radiation emitted by source **1404** and a susceptance material **1406** is included, within container **1405** that surrounds the mould **1402.** In the illustrated embodiment, the susceptance material **1406** is a granular particulate material comprised of particles of silicon carbide. A granular susceptance material is preferred in some applications as it allows suscepted heat to be applied intimately to the mould. In the illustrated embodiment, container **1405** is filled with particles **1406** of the susceptance material and mould **1402** is placed in the container so as to be partially or wholly immersed in granular susceptance material **1406.** By immersing mould **1402** in susceptance material **1406** not only is thermal energy efficiently transferred from the susceptance material **1406** to the surface of mould **1402,** but also mould **1402** is supported by susceptance material **1406,** thereby reducing the risk of the mould fracturing when loaded with metal powder **1403.**

## Claims

1. A method of forming a metal component from a powdered feed material (108), comprising the steps of:
creating a negative mould (104, 501) of a component from a ceramics material having a melting point that is higher than the melting point of said powdered feed material;
deploying said feed material of metal powder into said mould;
locating said mould in a vacuum chamber (1205) having an induction or microwave heating system, said heating system comprising a source of electromagnetic energy (1207, 1304, 1404) and a granular susceptance material; and
heating said mould using said heating system to a temperature higher than the melting point of the metal powder so as to melt said metal powder within the mould; wherein
said granular susceptance material absorbs the energy of the field generated by said source of electromagnetic energy and radiates infra-red energy towards the ceramic mould.

2. The method of claim 1, wherein said negative mould is built about a sacrificial positive model (102) of the component.

3. The method of claim 2, wherein said step of building said negative mould consists of adding a plurality of layers (304) to the outside of said positive model.

4. The method of claim 1, wherein said step of heating said mould using said heating system comprises the step of generating microwave energy.

5. The method of claim 1, wherein said granular susceptance material is comprised of particles (1406) of silicon carbide.

6. The method of claim 3, wherein said plurality of layers comprises a primary refractory slurry (301) that is inert to said powdered feed material.

7. The method of claim 3, wherein the plurality of layers are applied as an alternating wet slurry layer (301) followed by a substantially dry stucco layer (302) and said alternating slurry layers and stucco layers contain substantially similar ceramic material.

8. The method of claim 1, further comprising the step of feeding additional liquefied metal into said mould as said mould cools and the metal contained within said mould contracts.

9. The method of claim 8, further comprising the step of feeding said additional liquefied material into a feeder section (503) up to a head level to assist in forcing molten metal into the mould during cooling.

10. The method of claim 9, further comprising the step of providing an atmospheric core (505) to said feeder section and allowing gas trapped within said liquefied metal to escape via said atmospheric core.

11. An apparatus for forming a metal component from a powdered feed material (108), comprising:
a negative mould (104, 501) of a component comprised of a ceramics material having a melting point higher than the melting point of said powdered feed material contained therein; and
a vacuum chamber (1205) for receiving said mould, the vacuum chamber having an induction or microwave heating system, comprising a source of electromagnetic energy (1207, 1304, 1404) and a granular susceptance material, wherein
said granular susceptance material is configured to absorb the energy of the field generated by said source of electromagnetic energy and radiate infra-red energy towards the ceramic mould.

12. The apparatus of claim 11, further comprising a sacrificial positive model (102) of the component to be formed about which said negative mould is built.

13. The apparatus of claim 11, wherein said granular susceptance material is comprised of particles (1406) of silicon carbide.

14. The apparatus of claim 11, wherein said source of electromagnetic energy comprises a source of microwave radiation.

15. The apparatus of claim 11, wherein said negative mould is comprised of an alumina material having a high thermal conductivity.

16. The apparatus of claim 11, wherein the negative mould defines a component section (502) corresponding to the metal component being produced and a feeder section (503) for feeding additional liquefied metal into said component section as said mould cools and the metal contained within contracts.

17. The apparatus of claim 16, wherein said feeder section extends vertically upwards from said component section and comprises a head level, and the difference in height between the top of said component section and said head level is more than twice the height of said component section.

18. The apparatus of claim 16, wherein said feeder section has a first end adjoining said component section and a distal end extending therefrom and open to allow insertion of feed materials up to said head level.

19. The apparatus of claim 16, wherein said feeder section comprises an atmospheric core (505) that is porous to gasses for allowing gas trapped within the liquefied metal in said feeder section to escape.

## Patentansprüche

1. Eine Methode, eine Metallkomponente aus einem pulverisierten Aufgabematerial (108) zu formen, die die folgenden Schritte umfasst:
Erstellung einer Negativform (104, 501) einer Komponente aus einem Keramikmaterial, dessen Schmelzpunkt höher liegt als der Schmelzpunkt des besagten pulverisierten Aufgabematerials;
Einbringung des besagten Aufgabematerials aus Metallpulver in besagte Form;
Platzierung besagter Form in einer Vakuumkammer (1205), die ein Induktions- oder Mikrowellenheizsystem hat, wobei das besagte Heizsystem eine Quelle elektromagnetischer Energie (1207, 1304, 1404) und ein granulares Suszeptanzmaterial umfasst; und
Erhitzen besagter Form durch besagtes Heizsystem auf eine Temperatur, die höher als der Schmelzpunkt des Metallpulvers liegt, um besagtes Metallpulver in der Form zu schmelzen; wobei
besagtes granulares Suszeptanzmaterial die Energie des Feldes, das durch besagte Quelle elektromagnetischer Energie generiert wird, aufnimmt, und Infrarotenergie in Richtung der Keramikform ausstrahlt.

2. Die Methode aus Patentanspruch 1, wobei besagte Negativform um ein zerstörbares Positivmodell (102) der Komponente herum gebaut wird.

3. Die Methode aus Patentanspruch 2, wobei besagter Schritt des Baus besagter Negativform daraus besteht, der Außenseite des besagten Positivmodells eine Vielzahl an Schichten (304) hinzuzufügen.

4. Die Methode aus Patentanspruch 1, wobei besagter Schritt des Erhitzens besagter Form durch besagtes Heizsystem den Schritt der Generierung von Mikrowellenenergie umfasst.

5. Die Methode aus Patentanspruch 1, wobei besagtes granulares Suszeptanzmaterial aus Partikeln (1406) von Siliziumkarbid besteht.

6. Die Methode aus Patentanspruch 3, wobei besagte Vielzahl an Schichten einen primären feuerfesten Schlamm (301) umfasst, der gegenüber besagtem pulverisiertem Aufgabematerial träge ist.

7. Die Methode aus Patentanspruch 3, wobei die Vielzahl an Schichten als eine abwechselnde feuchte Schlammschicht (301), gefolgt von einer substantiell trockenen Stuckschicht (302), aufgetragen werden, und besagte abwechselnde Schlamm- und Stuckschichten enthalten substantiell ähnliches Keramikmaterial.

8. Die Methode aus Patentanspruch 1, die weiterhin den Schritt des Einbringens zusätzlichen geschmolzenen Metalls in besagte Form umfasst, da die besagte Form abkühlt und das Metall, das sich in besagter Form befindet, zusammenzieht.

9. Die Methode aus Patentanspruch 8, die weiterhin den Schritt des Einbringens besagten zusätzlichen geschmolzenen Materials in ein Abgangsfeld (503) bis zu einer Kopfhöhe umfasst, um dabei zu helfen, geschmolzenes Metall während des Abkühlens in die Form zu zwingen.

10. Die Methode aus Patentanspruch 9, die weiterhin den Schritt der Zurverfügungstellung eines atmosphärischen Kerns (505) für besagtes Abgangsfeld umfasst, und es in besagtem geschmolzenem Metall eingeschlossenen Gas ermöglicht, über besagten atmosphärischen Kern zu entweichen.

11. Ein Apparat zur Erstellung einer Metallkomponente aus einem pulverisierten Aufgabematerial (108), der folgendes umfasst:
eine Negativform (104, 501) einer Komponente aus einem Keramikmaterial, dessen Schmelzpunkt höher liegt als der Schmelzpunkt des besagten pulverisierten Aufgabematerials darin; und
eine Vakuumkammer (1205) zur Aufnahme besagter Form, wobei die Vakuumkammer ein Induktions- oder Mikrowellenheizsystem hat, das eine Quelle elektromagnetischer Energie (1207, 1304, 1404) und ein granulares Suszeptanzmaterial umfasst, wobei
besagtes granulares Suszeptanzmaterial so konfiguriert ist, die Energie des Feldes, das durch besagte Quelle elektromagnetischer Energie generiert wird, aufnimmt, und Infrarotenergie in Richtung der Keramikform ausstrahlt.

12. Der Apparat aus Patentanspruch 11, der weiterhin ein zerstörbares Positivmodell (102) der zu formenden Komponente umfasst, um die besagte Negativform herum gebaut wird.

13. Der Apparat aus Patentanspruch 11, wobei besagtes granulares Suszeptanzmaterial aus Partikeln (1406) von Siliziumkarbid besteht.

14. Der Apparat aus Patentanspruch 11, wobei besagte Quelle elektromagnetischer Energie eine Quelle für Mikrowellenstrahlung umfasst.

15. Der Apparat aus Patentanspruch 11, wobei besagte Negativform aus einem Aluminiummaterial besteht, das eine hohe thermische Leitfähigkeit besitzt.

16. Der Apparat aus Patentanspruch 11, wobei die Negativform einen Komponentenbereich definiert (502), der mit der zu produzierenden Metallkomponente und einem Abgangsfeld (503) zum Einbringen zusätzlichen geschmolzenen Metalls in besagten Komponentenbereich übereinstimmt, da sich besagte Form abkühlt und das darin enthaltene Metall sich zusammenzieht.

17. Der Apparat aus Patentanspruch 16, wobei besagtes Abgangsfeld sich von besagtem Komponentenbereich aus vertikal nach oben erstreckt und eine Kopfhöhe umfasst, und der Höhenunterschied zwischen der Spitze des besagten Komponentenbereichs und der besagten Kopfhöhe ist mehr als die doppelte Höhe des besagten Komponentenbereichs.

18. Der Apparat aus Patentanspruch 16, wobei besagtes Abgangsfeld ein erstes Ende hat, das an besagten Komponentenbereich angrenzt, und ein distales Ende, das sich von dort aus erstreckt und sich öffnet, um das Einbringen von Aufgabematerialien bis zur besagten Kopfhöhe zu ermöglichen.

19. Der Apparat aus Patentanspruch 16, wobei besagtes Abgangsfeld einen atmosphärischen Kern (505) umfasst, der für Gase durchlässig ist, um in geschmolzenem Metall in besagtem Abgangsfeld eingeschlossenes Gas entweichen zu lassen.

## Revendications

1. Méthode de formation d'un composant métallique à partir d'une matière première pulvérulente (108), comprenant les étapes suivantes :
création d'un moule négatif (104, 501) d'un composant, réalisé avec un matériau céramique dont le point de fusion est supérieur au point de fusion de ladite matière première pulvérulente ;
déploiement de ladite matière première de poudre métallique dans ledit moule ;
positionnement dudit moule dans une chambre à vide (1205) possédant un système de chauffage à induction ou à microondes, ledit système de chauffage possédant une source d'énergie électromagnétique (1207, 1304, 1404) et une matière de susceptance granulaire ; et
chauffage dudit moule à l'aide dudit système de chauffage à une température supérieure au point de fusion de la poudre métallique, de façon à opérer la fusion de ladite poudre métallique au sein du moule ;
ladite matière de susceptance granulaire absorbant l'énergie du champ généré par ladite source d'énergie électromagnétique, et rayonnant de l'énergie infrarouge vers le moule de céramique.

2. Méthode selon la revendication 1, ledit moule négatif étant réalisé autour d'une maquette positive sacrificielle (102) du composant.

3. Méthode selon la revendication 2, ladite étape de réalisation dudit moule négatif comportant l'adjonction d'une pluralité de couches (304) sur l'extérieur de ladite maquette positive.

4. Méthode selon la revendication 1, ladite étape de chauffage dudit moule à l'aide dudit système de chauffage comportant l'étape de génération d'énergie de microondes.

5. Méthode selon la revendication 1, ladite matière de susceptance granulaire étant composée de particules (1406) de carbure de silicium.

6. Méthode selon la revendication 3, la pluralité de couches comprenant une boue réfractaire primaire (301) inerte à ladite matière première pulvérulente.

7. Méthode selon la revendication 3, la pluralité de couches étant appliquées en alternant une couche de boue humide (301) avec une couche de stuc substantiellement sèche (302), et lesdites couches de boue humide s'alternant avec des couches de stuc contenant une matière céramique substantiellement similaire.

8. Méthode selon la revendication 1, comprenant en outre l'étape d'introduction d'un métal liquéfié additionnel dans ledit moule, au fur et à mesure que ledit moule se refroidit et le métal contenu dans ledit moule se contracte.

9. Méthode selon la revendication 8, comprenant en outre l'étape d'introduction ledit métal liquéfié additionnel dans une section d'alimentation (503) jusqu'à un niveau de tête, afin de contribuer à l'introduction forcée de métal en fusion dans le moule au cours du refroidissement.

10. Méthode selon la revendication 9, comprenant en outre l'étape de fourniture d'un noyau atmosphérique (505) à ladite section d'alimentation et d'évacuation du gaz piégé dans ledit métal liquéfié via ledit noyau atmosphérique.

11. Appareil pour la formation d'un composant métallique à partir d'une matière première pulvérulente (108), comprenant :
un moule négatif (104, 501) d'un composant, réalisé avec un matériau céramique dont le point de fusion est supérieur au point de fusion de ladite matière première pulvérulente contenue dans celui-ci ; et
une chambre à vide (1205) pour la réception dudit moule, la chambre à vide possédant un système de chauffage à induction ou à microondes, comprenant une source d'énergie électromagnétique (1207, 1304, 1404) et une matière de susceptance granulaire, dans laquelle
ladite matière de susceptance granulaire est configurée pour absorber l'énergie du champ généré par ladite source d'énergie électromagnétique, et rayonner de l'énergie infrarouge vers le moule de céramique.

12. Appareil selon la revendication 11, comprenant en outre une maquette positive sacrificielle (102) du composant à former, autour de laquelle est réalisé ledit moule négatif.

13. Appareil selon la revendication 11, ladite matière de susceptance granulaire étant composée de particules (1406) de carbure de silicium.

14. Appareil selon la revendication 11, ladite source d'énergie électromagnétique comprenant une source de rayonnement microondes.

15. Appareil selon la revendication 11, ledit moule négatif étant composé d'un matériau d'alumine présentant une conductivité thermique élevée.

16. Appareil selon la revendication 11, ledit moule négatif définissant une section du composant (502) correspondant au composant métallique en cours de production, et une section d'alimentation (503) pour l'introduction d'un métal liquéfié dans ladite section du composant au fur et à mesure que ledit moule se refroidit et le métal contenu dans ledit moule se contracte.

17. Appareil selon la revendication 16, ladite section d'alimentation s'étendant verticalement vers le haut depuis ladite section du composant, et comprenant un niveau de tête, et la différence de hauteur entre le dessus ladite section du composant et ledit niveau de tête mesurant plus du double de la hauteur de ladite section du composant.

18. Appareil selon la revendication 16, ladite section d'alimentation comprenant un premier bout contigu à ladite section du composant, et une extrémité distale s'étendant depuis celle-ci, et ouverte pour permettre l'insertion de matières premières jusqu'audit niveau de tête.

19. Appareil selon la revendication 16, ladite section d'alimentation comprenant un noyau atmosphérique (505) poreux aux gaz, afin de permettre l'échappement du gaz piégé au sein du métal liquéfié dans ladite section d'alimentation.
